

May 29, 1956

P. M. MADER  
REMOVING SILVER AND SILVER HALIDE  
FROM PHOTOGRAPHIC ELEMENTS  
Filed April 1, 1954

2,748,000



PAUL M. MADER  
INVENTOR.

BY *Daniel L. Mayne*  
*W.H. McGowen*  
ATTORNEY & AGENT

# United States Patent Office

2,748,000  
Patented May 29, 1956

## 1

2,748,000

### REMOVING SILVER AND SILVER HALIDE FROM PHOTOGRAPHIC ELEMENTS

Paul M. Mader, Rochester, N. Y., assignor to Eastman Kodak Company, Rochester, N. Y., a corporation of New Jersey

Application April 1, 1954, Serial No. 420,302

15 Claims. (Cl. 95—88)

This invention relates to the removal of silver and silver halide from photographic elements. A variety of agents for these purposes are known and the selection depends on the requirements of the particular process involved. Thus in conventional development of a silver halide latent image to a black silver image it is desired to remove residual silver halide without attacking developed silver. This can be done with thiosulfate or thiocyanate solutions. In other instances it is desired to remove a developed silver image without affecting residual undeveloped silver halide, for example, in direct positive development where negative metallic silver is removed before the residual silver halide is developed to the silver positive image. The removal is effected with an oxidizing bath, such as potassium dichromate-sulfuric acid, or potassium permanganate-sulfuric acid solution. These bleaches convert the silver to soluble silver salts which diffuse out of the emulsion layer, without attacking the residual silver halide.

In still other cases it may be desirable to remove both silver and silver halide as is true in some color processes. This may be done with a potassium cyanide solution or with an oxidizing bleach solution, such as dichromate, ferricyanide, or quinone, containing or followed by a silver salt solvent to ensure removal of both the oxidized image silver and the residual silver halide.

It is difficult to find otherwise satisfactory silver halide solvents of sufficient stability for use in the presence of the strongly oxidizing bleach compounds. There are also instances where it is advantageous to be able to remove the image silver along with a distinct part of the residual silver halide, for example, the silver chloride, while leaving comparatively unaffected another portion comprising, for example, silver bromide.

I have discovered a group of related compounds which are silver salt solvents and useful for the removal of silver halide from photographic layers. Some of them compare favorably with alkali thiosulfates and thiocyanates in the orthodox fixing process and in addition have the unusual and beneficial properties of exceptional stability in solutions not only to acids and alkalies but to the oxidizing agents commonly used in combination bleaching and fixing baths for the removal of both silver and silver salts from photographic layers. Furthermore, they show a selectivity or specificity in solvent activity for different silver salts commonly used in photographic layers.

These compounds are sulfur-containing dibasic acids of the general formula:

$\text{HOOC}-\text{CH}_2-(\text{S}-\text{CH}_2\text{CH}_2)_n-\text{S}-\text{CH}_2-\text{COOH}$   
in which  $n$  1, 2, or 3 alkali metal or ammonium salts thereof.

The following compounds and their water-soluble salts are therefore contemplated for use in my invention:

1. Ethylene-bis-thioglycolic acid

$\text{HOOC}-\text{CH}_2-\text{S}-(\text{CH}_2)_2-\text{S}-\text{CH}_2-\text{COOH}$

2. 3,6,9-trithiahexadecanedioic acid

$\text{HOOC}-\text{CH}_2-(\text{S}-\text{CH}_2-\text{CH}_2)_2-\text{S}-\text{CH}_2-\text{COOH}$

3. 3,6,9,12-tetrathiatetradecanedioic acid

$\text{HOOC}-\text{CH}_2-(\text{S}-\text{CH}_2-\text{CH}_2)_3-\text{S}-\text{CH}_2-\text{COOH}$

## 2

These compounds are useful as fixing agents to remove silver halide from hydrophilic organic colloid layers of photographic elements. Compounds 2 and 3 are not very soluble in water in the acid form and are preferably used as the salts, e. g., the sodium salt. The ethylene-bis-thioglycolic acid may be used either in acid or salt form. It has the advantageous property of dissolving silver chloride at a much faster rate than it dissolves silver bromide, so that it can be used for the selective removal of the chloride in the presence of the bromide. Sodium chloride, sodium sulfite, and certain other silver halide solvents show a similar selective fixing action, but they have one or more shortcomings which make them impractical in many applications, e. g., slow rate of dissolving, instability in the presence of oxidizing agents, low activity, etc.

Compounds 2 and 3 are much more rapid fixing agents for silver halide than ethylene-bis-thioglycolic acid. The sodium salt of Compound 2, for example, fixes silver bromide in about one third the time required for an equimolecular concentration of ethylene-bis-thioglycolic acid. The sodium salt of Compound 3 at 0.05 molar concentration clears a simple silver bromide emulsion in less than half the time required for sodium thiosulfate solution at the same molar concentration. Similarly a solution of the sodium salt of Compound 3 is a faster acting fixing agent for silver bromide than the sodium salt of Compound 2. A 0.05 molar solution of the sodium salt of Compound 3 fixed a silver bromide emulsion in one minute and forty seconds at 75° F.

30 The homologous compounds of ethylene-bis-thioglycolic acid in which the ethylene chain between the two sulfur atoms is replaced with methylene, propylene, tetramethylene, or higher alkylene groupings form considerably weaker complexes than does the ethylene derivative Compound 1, and hence their potential value as fixing agents does not approach that of ethylene-bis-thioglycolic acid.

35 The exceptional stability of the fixing agents, Compounds 1, 2, and 3, becomes apparent when they are used in combination bleaching and fixing solutions for the removal of silver from emulsions or other silver colloid layers, such as colloidal silver filter layers in photographic elements. This can, of course, be done by the conventional method of first oxidizing the silver to a silver halide by treatment with ferricyanide-bromide, or the like, and

40 then removing the silver halide thus formed in a separate fixing bath, such as the conventional hypo solution. It is much more convenient to accomplish the oxidizing and bleaching operation and the solution of the silver salt in one step. A number of one bath solutions for this purpose are known, e. g., a reducer such as ferrocyanide-hypo solution might be used. Such baths, however, are usually not sufficiently stable. My compounds enable the preparation of a combined bleaching and fixing solution of good stability, excellent solvent properties for both silver and silver halide, and capable of formula and use modifications to permit removal of the silver and all the residual silver halide or of the silver along with selective removal of the silver chloride without appreciable attack on the silver bromide.

45 60 Accordingly, aqueous solutions containing a mixture of a silver oxidizing agent such as quinone or an alkali metal ferricyanide and one of the above sulfur-containing dibasic acids are very effective in the removal of silver from hydrophilic colloid layers of photographic elements.

65 A particular application of one of the dibasic sulfur compounds of the invention, ethylene-bis-thioglycolic acid, is in the simultaneous removal of a silver image and silver chloride from a system containing both silver chloride and silver bromide as described in more detail in the following examples. In this case it is found that a solution of a mixture of an oxidizing agent, e. g., quinone, and the dibasic sulfur compound serves not only to dis-

solve the silver image but the ability of the ethylene-bis-thioglycolic acid to selectively remove silver chloride from the system in the presence of silver bromide is not impaired by the presence of the oxidizing agent.

An important advantage of the mentioned bleaching-fixing solutions containing oxidizing agent and one of the sulfur-containing dibasic acids lies in the high stability of the solutions. For example, a solution containing ethylene-bis-thioglycolic acid and quinone was found to lose none of its power for fixing silver chloride or removing silver from a colloid layer after standing for eight days although the solution had darkened appreciably. Similarly, a solution of ethylene-bis-thioglycolic acid and potassium ferricyanide at a pH of 6.5 which had been stored 50 days still fixed silver chloride and oxidized silver at the same rate as when the solution was first prepared. Also, the solution did not become discolored over this period of time.

The compositions of the invention containing a mixture of one of the dibasic sulfur compounds and an oxidizing agent, such as ethylene-bis-thioglycolic acid and potassium ferricyanide, find use as a "reducer" for removing metallic silver slowly from a photographic image in a manner similar to "Farmer's Reducer" as shown in the following examples. In this case, when ferricyanide is used as the oxidizing agent, the concentration is maintained at a low level to prevent formation of silver ferrocyanide in the image.

The accompanying drawings illustrate in cross-sectional view the appearance of a color film at various stages in the formation of colored images in the film and the selective removal of silver and silver chloride from the film in the presence of an exposed silver bromide emulsion.

My invention is described in more detail in the following examples with reference to the accompanying drawings.

#### EXAMPLE I

A two-layer color film was prepared as described in U. S. Patent 2,490,751 and shown in Stage 1 of the accompanying drawings as having a support 10 carrying a gelatino silver halide emulsion layer 11 containing a mixture of a green-sensitive silver chloride emulsion, magenta coupler and a blue-sensitive silver bromide emulsion of the internal latent image type. Coated thereon is a red-sensitive silver chloride emulsion layer 12 containing a cyan coupler. The film was exposed to a colored subject and samples were processed in the following processes, Process A representing a process using the conventional bleaching and selective fixing steps and Process B incorporating the combined fixing-bleaching step of the invention.

#### Process A (70° F.)

|               | Minutes |
|---------------|---------|
| Color develop | 12      |
| Stop          | 1       |
| Wash          | 5       |
| Bleach        | 10      |
| Wash          | 5       |
| Selective fix | 9       |
| Wash          | 10      |
| Develop (I)   | 5       |
| Fix (I)       | 15      |
| Wash          | 10      |

#### Process B (70° F.)

|               | Minutes |
|---------------|---------|
| Color develop | 12      |
| Stop          | 1       |
| Wash          | 5       |
| Fix-bleach    | 15      |
| Wash          | 5       |
| Develop (II)  | 5       |
| Rinse         |         |
| Fix (II)      | 3       |
| Wash          | 10      |

The processing solutions had the following compositions:

#### Color developer:

|    |                                                   |       |    |
|----|---------------------------------------------------|-------|----|
| 5  | Sodium hexametaphosphate                          | grams | 1  |
|    | Na <sub>2</sub> SO <sub>3</sub>                   | do    | 12 |
|    | 2-amino-5-diethylaminotoluene hydrochloride       | do    | 3  |
| 10 | Na <sub>2</sub> CO <sub>3</sub> ·H <sub>2</sub> O | do    | 20 |
|    | KBr                                               | do    | 2  |
|    | H <sub>2</sub> O                                  | liter | 1  |

#### Stop bath:

|    |                       |       |    |
|----|-----------------------|-------|----|
| 15 | Acetic acid (glacial) | grams | 20 |
|    | H <sub>2</sub> O      | liter | 1  |

#### Bleach bath:

|    |                                               |       |   |
|----|-----------------------------------------------|-------|---|
| 15 | K <sub>2</sub> Cr <sub>2</sub> O <sub>7</sub> | grams | 2 |
|    | H <sub>2</sub> O                              | liter | 1 |
|    | H <sub>2</sub> SO <sub>4</sub> to make pH=1.9 |       |   |

#### Selective fix:

|    |                                 |       |     |
|----|---------------------------------|-------|-----|
| 20 | Na <sub>2</sub> SO <sub>3</sub> | grams | 100 |
|    | H <sub>2</sub> O                | liter | 1   |

#### Developer I:

|    |                                  |       |      |
|----|----------------------------------|-------|------|
| 25 | Monomethyl-p-aminophenol sulfate | grams | 2.2  |
|    | Na <sub>2</sub> SO <sub>3</sub>  | do    | 96.0 |
|    | Hydroquinone                     | do    | 8.8  |
|    | Na <sub>2</sub> CO <sub>3</sub>  | do    | 48.0 |
|    | KBr                              | do    | 5.0  |
|    | KI                               | do    | 6.0  |
|    | NaOH                             | do    | 10.0 |
|    | H <sub>2</sub> O                 | liter | 1    |

#### Developer II:

|    |                                               |       |      |
|----|-----------------------------------------------|-------|------|
| 30 | Monomethyl-p-aminophenol sulfate              | grams | 2.2  |
|    | Na <sub>2</sub> SO <sub>3</sub>               | do    | 96.0 |
|    | Hydroquinone                                  | do    | 8.8  |
|    | Na <sub>2</sub> CO <sub>3</sub>               | do    | 48.0 |
|    | KBr                                           | do    | 5.0  |
|    | Na <sub>2</sub> S <sub>2</sub> O <sub>3</sub> | do    | 5.0  |
|    | H <sub>2</sub> O                              | liter | 1    |

#### Fix I:

|    |                                                               |       |     |
|----|---------------------------------------------------------------|-------|-----|
| 35 | (NH <sub>4</sub> ) <sub>2</sub> S <sub>2</sub> O <sub>3</sub> | grams | 250 |
|    | Na <sub>2</sub> SO <sub>3</sub>                               | do    | 10  |
|    | H <sub>2</sub> O to make 1 liter                              |       |     |

#### Fix II:

|    |                                  |       |       |
|----|----------------------------------|-------|-------|
| 40 | Water, about 125° F. (50° C.)    | cc    | 600   |
|    | Sodium thiosulfate, pentahydrate | grams | 240.0 |
|    | Sodium sulfite, desiccated       | do    | 15.0  |
|    | Acetic acid, 28%                 | cc    | 48.0  |
|    | Boric acid, crystals             | grams | 7.5   |
|    | Potassium alum                   | do    | 15.0  |
|    | Cold water to make 1.0 liter     |       |       |

#### Fix-bleach:

|    |                                |       |     |
|----|--------------------------------|-------|-----|
| 45 | Ethylene-bis-thioglycolic acid | grams | 16  |
|    | Quinone                        | do    | 3.5 |
|    | H <sub>2</sub> O               | liter | 1   |

Accordingly, in Process A, color development forms silver and magenta and cyan dye images in layers 11 and 12 of the film, the bleach and selective fixing steps removing the silver images and residual silver chloride from the film, leaving the dye images and exposed silver bromide emulsion in the film. Subsequent development with the developer I yields a silver image of the blue sensation in layer 11. This developer can, of course, be replaced by a "solvent" type of yellow image-forming color developer such as shown in U. S. Patent 2,490,791 to yield a yellow dye image in layer 11 together with the previously developed magenta dye image and the cyan image in layer 12.

Process B embodying the combined fixing-bleaching step of the invention is illustrated in the accompanying drawings wherein the exposed element of Stage 1 of the drawings described above is shown in Stage 2 of the drawings following color development, stop bath and

washing steps, as containing magenta and cyan dye images as well as silver images in layers 11 and 12 and the undeveloped blue-sensitive latent image in silver bromide in layer 11, residual silver chloride remaining in layers 11 and 12. As the result of treatment with the fixing-bleaching bath of the invention, the element appears as described in Stage 3 of the drawings, the silver images as well as the residual silver chloride in layers 11 and 12 having been removed leaving the magenta and cyan dye images in layers 11 and 12 and the latent image in silver bromide in layer 11.

Following development of the element of the third stage of the drawings with the black-and-white "solvent" developer II, or a solvent type of yellow color-forming developer, such as shown in U. S. Patent 2,490,751, the element contains a silver, or silver and yellow dye image and the magenta dye image in layer 11 as well as a cyan dye image in layer 12 as described in Stage 4 of the drawings. In case a solvent type of color developer has been used in the last development step, the resultant silver image can be removed with the fixing-bleach bath of the invention or by conventional methods, leaving only cyan, magenta and yellow dye images in the film.

When sensitometric curves of the subtractively colored dye images formed in the conventional Process A were compared with the curves of the dye images formed in Process B of the invention, it was found that the comparable dye images of the two processes had the same contrast, and other sensitometric characteristics of the element of Process B were favorable. In particular, the desired contrast and other characteristics were obtained in Process B in the image corresponding to the blue light exposure.

A fixing-bleaching bath containing about 2 to 10 grams of potassium ferricyanide and about 16 grams of ethylene-bis-thioglycolic acid per liter at a pH of about 6.5 can be used for the removal of silver images in processes such as that described in the above example. However, the rate of removal of silver is somewhat lower than when the quinone-containing fixing-bleaching solution is used.

In those processes such as present-day color development processes, in the final stages of which it is desired to remove silver images and all residual silver halide in the presence of color-developed dye images, very satisfactory results will be obtained with a fixing-bleach bath containing an alkali salt of Compound 3 above in conjunction with ferricyanide.

#### EXAMPLE 2

The mentioned use of the sulfur-containing dibasic acids in conjunction with an oxidizing agent as a "reducer" for the slow removal of silver from silver images in a manner similar to Former's reducer is demonstrated by first forming a silver image in a light-sensitive film or paper product followed by fixing in the usual manner. The film is then treated in a solution of the following composition:

|                                     |       |       |       |
|-------------------------------------|-------|-------|-------|
| Ethylene-bis-thioglycolic acid      | ----- | grams | 4.0   |
| Water                               | ----- | cc    | 250.0 |
| Sodium hydroxide to bring pH to 6.5 | ----- |       |       |
| Potassium ferricyanide              | ----- | grams | 0.75  |

Treatment of a silver image developed in a high-speed negative film with this solution at 70° C. for 30 seconds, 1 minute, 3 minutes and 8 minutes, gave silver densities as follows:

|                        |       |      |
|------------------------|-------|------|
| 1. Untreated image     | ----- | 1.85 |
| 2. 30-second treatment | ----- | 1.76 |
| 3. 1-minute treatment  | ----- | 1.65 |
| 4. 3-minute treatment  | ----- | 1.42 |
| 5. 8-minute treatment  | ----- | 0.8  |

After holding the above solution for 49 days, the solution gave a silver density of 0.94 at Log E 3.6 when the same silver image was "reduced."

The activity of the reducer solution appears to be intermediate between a proportional and a subtractive reducer solution.

The following example illustrates the use of Compound 3 for the removal of silver and silver halide from photographic elements.

#### EXAMPLE 3

A multilayer product having blue-, green- and red-sensitive gelatin emulsion layers superposed in that order on a paper base was provided. The emulsion layers contained dispersions of color-forming couplers for forming subtractively colored dye images of colors complementary to the sensitivity of the respective emulsion layers. The paper was exposed in the usual manner to a color negative and developed 8 minutes in a conventional color developing solution containing a primary aromatic amino silver halide developing agent to obtain silver and dye images in the emulsion layers.

After color development the paper was treated 1½ minutes with a 1% acetic acid stop bath followed by a 4 minute wash and 10 minutes with a fix-bleach bath 0.05 molar in sodium-3,6,9,12-tetrathiatetradecanedioate and containing 15 grams of potassium ferricyanide per liter (pH=6.5). The silver and silver halide were thus removed and results were obtained comparable to the conventional use of ferricyanide or quinone bleach solutions followed by hypo. The pronounced stability of the fix-bleach bath of the invention was evident.

What I claim is:

1. A fixing-bleach composition for silver halide emulsion layers, comprising an aqueous solution of a mixture of (1) a member of the class consisting of quinone and an alkali metal ferricyanide, and (2) a compound having the general formula



wherein  $n$  represents a positive integer of from 1 to 3 and alkali metal and ammonium salts thereof.

2. A fixing-bleach composition for silver halide emulsion layers, comprising an aqueous solution of a mixture of quinone and ethylene-bis-thioglycolic acid.

3. A fixing-bleach composition for silver halide emulsion layers, comprising an aqueous solution of a mixture of potassium ferricyanide and ethylene-bis-thioglycolic acid.

4. A fixing-bleach composition for silver halide emulsion layers, comprising an aqueous solution of a mixture of potassium ferricyanide and sodium 3,6,9,12-tetrathiatetradecanedioate.

5. A process for the removal of silver from photographic elements which comprises treating a supported hydrophilic organic colloid layer containing silver with an aqueous solution of a mixture of (1) a member of the class consisting of quinone and an alkali metal ferricyanide, and (2) a compound having the general formula



wherein  $n$  represents a positive integer of from 1 to 3 and alkali metal and ammonium salts thereof.

6. A process for the removal of silver from photographic elements which comprises treating a supported hydrophilic organic colloid layer containing silver with an aqueous solution of a mixture of quinone and ethylene-bis-thioglycolic acid.

7. A process for the removal of silver from photographic elements which comprises treating a supported hydrophilic organic colloid layer containing silver with an aqueous solution of a mixture of potassium ferricyanide and ethylene-bis-thioglycolic acid.

8. A process for the removal of silver from photographic elements which comprises treating a supported hydrophilic organic colloid layer containing silver with an aqueous solution of a mixture of potassium ferricyanide and sodium 3,6,9,12-tetrathiatetradecanedioate.

9. A process for the selective removal of silver chlo-

ride from a photographic emulsion layer in the presence of an emulsion layer containing silver bromide, which comprises treating the silver chloride in the presence of the silver bromide with an aqueous solution of ethylene-bis-thioglycolic acid, until the silver chloride has been removed leaving silver bromide in an emulsion layer.

10. A process for the removal of silver from a photographic element containing a silver image, silver chloride and silver bromide which comprises treating said element with an aqueous solution of a mixture of quinone and ethylene-bis-thioglycolic acid until the silver and silver chloride have been removed leaving silver bromide in the element.

11. A process for the removal of a silver image from a photographic element containing a silver image, silver chloride and silver bromide which comprises treating said element with an aqueous solution of a mixture of quinone and ethylene-bis-thioglycolic acid until the silver and silver chloride have been removed leaving silver bromide in the element.

12. A process for the removal of silver halide from a hydrophilic-organic colloid photographic emulsion layer containing silver halide which comprises treating said layer with an aqueous solution of a compound having the general formula



wherein  $n$  represents a positive integer of from 1 to 3 and alkali metal and ammonium salts thereof.

13. A process for the removal of silver halide from a hydrophilic organic colloid photographic emulsion layer containing silver halide which comprises treating said layer with an aqueous solution of sodium 3,6,9-trithiahen-decanedioate.

14. A process for the removal of silver halide from a hydrophilic organic colloid photographic emulsion layer containing silver halide which comprises treating said layer with an aqueous solution of sodium 3,6,9,12-tetrathiahexadecanedioate.

15. A process for the removal of silver chloride from a hydrophilic organic colloid photographic emulsion layer containing silver halide which comprises treating said layer with an aqueous solution of ethylene-bis-thioglycolic acid.

References Cited in the file of this patent

UNITED STATES PATENTS

2,331,678 Hanson ----- Oct. 12, 1943